

Patented June 25, 1929.

1,718,548

# UNITED STATES PATENT OFFICE.

ALFRED ENGELHARDT, OF WIESDORF, NEAR COLOGNE-ON-THE-RHINE, GERMANY, AS-  
SIGNOR TO I. G. FARBNENINDUSTRIE AKTIENGESELLSCHAFT, OF FRANKFORT-ON-  
THE-MAIN, GERMANY.

## PROCESS FOR THE DEGREASING OF RAW WOOL AND OTHER TEXTILE FIBERS.

No Drawing. Application filed February 10, 1927, Serial No. 167,358, and in Germany March 12, 1926.

The present invention concerns the degreasing of raw wool or other textile fibers by the application of cyclohexanone or its homologues.

5 For some considerable time attempts have been made to effect the washing of wool by the aid of organic fat solvents instead of by the hitherto employed method of using soap exclusively, since it has been found that in this 10 manner the wool fiber is protected to a greater extent and also a more valuable wool fat is obtained. However, this problem hitherto had not been solved successfully from a technical and economical point of view, since none 15 of the solvents proposed for this purpose possesses all the properties required by a rational large scale operation.

The properties of such a solvent should be as follows:

20 It should possess a high solvent capacity for wool fat and wool wax at ordinary temperature and should be sufficiently mobile. It should be stable towards boiling dilute alkalies. It is, further, indispensable for the 25 safety of the process that the solvent should not emit any easily inflammable vapors and should not give rise to injurious physiological action. For economy in its use it is absolutely essential that it should not incur losses due to 30 too great volatility, neither should it have a corrosive action on metals. It is also of great importance that the solvent should be to a certain extent soluble in water, in order to facilitate a simple execution of the washing 35 process.

The solvents hitherto proposed, such as, for example, benzene, carbon tetrachloride, trichlorethylene, ether, acetone, acetic acid ester and carbonic acid ester of methanol and ethyl 40 alcohol, do not satisfy these fundamental requirements.

The present invention is based on the discovery of the fact that cyclohexanone and its homologues, such as, for example, methyl cyclohexanone, possess all the above properties and are thus excellently suited to application as de-greasing agents for wool. For example, the essential characteristics of cyclohexanone are as follows:

45 Its capacity for dissolving wool fat and wool wax at ordinary temperature equals that of benzene, to which it also corresponds as regards mobility. It boils at 155° C., and the vapor tension at ordinary temperature is no

higher than that of water. Since the flash 55 point is 39° C. (the flash point of benzene being 8° C.), the technical application involves practically no danger owing to inflammability. Cyclohexanone does not exert an unfavorable physiological action under the 60 conditions obtaining in actual practice. No substantial losses are to be feared from vaporization and it does not decompose on heating with dilute alkaline solutions. One part of cyclohexanone dissolves in about 11 parts of 65 water, from which solution it can be isolated by salting out, or by extraction with oils. The solubility in water effects an easy and efficient washing of the wool with the result that any adherent residues of solvent are completely removed after extraction. 70

By the application of cyclohexanone as solvent a soft pure wool is produced, which retains its original curly nature and is equivalent in quality to the best products obtained 75 from raw wool by extraction with other organic solvents.

The invention will be more fully described by reference to the following, and subsequent, examples:

80 *Example 1.*—The suint wool is freed from dust by beating and loosely compressed by a punch or plunger in cylindrical containers about 4 ft. in diameter and 15 ft. high, where-in the wool is carried on metal screen plates located about 10 cm. above the floor of the 85 container. Cyclohexanone is then passed from below into the container and passes upwardly through the wool and is saturated with wool fat, whereby the solvent takes up 90 wool fat up to 9% by weight of wool fat. The wool fat solution passes from the extraction apparatus through a lateral discharge. The wool fat is obtained from the saturated 95 wool fat solution in known manner by distilling off the cyclohexanone at reduced pressure, while the solutions having a low wool fat content and obtained at the end of the extraction are further enriched on further extraction. When the wool fat content of the 100 cyclohexanone passing from the washing apparatus has dropped to 0.2% by weight, extraction is terminated. The cyclohexanone is 105 passed from the apparatus below, whereby the wool is strongly compressed by the plunger. The wool is then loosened by raising the plunger and the cyclohexanone adhering thereto is washed therefrom with wa-

ter in the same manner as the wool fat was previously dissolved out, whereby the wool is repeatedly compressed and loosened. The suint salts are also dissolved out of the wool 5 during the operation described.

After this extraction procedure the wool is washed moderately with soap solution to remove the last traces of dirt, rinsed moderately with water, and then dried by hot air.

10 In such cases where a particularly mild extraction of open wool is required in order to retain a slight amount of fat in the capillaries of the cellular fibers, there may be employed cyclohexanone, or a homologue there-  
 15 of, containing a regulated, predetermined small quantity of fat, as, for example, wool fat. For the purpose of the present invention, by a predetermined small quantity is meant a content of the order of one percent  
 20 or thereabouts. Or, there may be employed a mixture comprising cyclohexanone and other water-soluble organic solvents, the latter solvents having only a relatively small solvent capacity for wool fat and particu-  
 25 larly for wool wax; e. g., alcohol, glycerin or the like.

*Example 2.*—Beaten Merino suint wool is passed in counter-current to a solution of 0.2% by weight of wool fat in a mixture of 30 80 parts by weight of methyl-cyclohexanone and 20 parts by weight of 96% ethyl alcohol, in three "Leviathan" washers, whereby the wool fat is removed from the wool and a solution containing about 6% wool fat is obtained. The wool fat is separated from this 35 solution by distilling off the solvent. After the fat is removed, the wool is freed of the adhering solvent residue and of the suint salts by washing with water in two connected 40 "Leviathan" washers. The wool is treated with a dilute soap solution to remove the last traces of dirt, rinsed with clear water, and then dried with hot air.

It will depend entirely on the particular 45 kind of wool, whether the raw wool is first subjected to washing with an aqueous liquid, as, for example, water, or an ordinary aqueous soap solution, in order to extract the potassium salts, and then is further extracted 50 in a moist or dry condition with cyclohexanone alone or in admixture with other organic solvents, or whether the raw wool is subjected to extraction direct, and, if necessary, is afterwards subjected to treatment 55 with an aqueous liquid. In all these cases, cyclohexanone achieves a thorough de-greasing and produces a soft wool which is not matted or stringy.

*Example 3.*—Suint wool is freed from dust 60 by beating, loosened up, and the salt removed by allowing water to trickle thereon while it is advanced on a perforated conveyor band. After expressing the greater quantity of the water, the wool passes through three "Leviathan" washers, through which methyl-cyclo-

hexanone is passed in counter-current to the moving wool. The solution passing from the first washer has about 8% by weight of wool fat, which is separated from the solution by distilling off the methyl-cyclohexanone at reduced pressure. The wool, from which the fat has been removed, on passing from the third washer, is freed from solvent by washing with water in two other washers and expressing, moderately soaped to remove the 75 last traces of dirt, the soap rinsed out, and the washed wool is dried.

The wool fat is recovered from the wool fat solutions in the customary manner by distilling off the cyclohexanone under ordinary or reduced pressure as a residue of yellowish coloration. The solvent residues adhering to the wool after the extraction can be replaced by water according to the known method for carbon tetrachloride extraction, the process being of course particularly easily effected owing to the water solubility of the cyclohexanone.

The washing process with cyclohexanone is carried out on the large scale using the apparatus customary for wool washing. When the process is subject to being interrupted, as, for example, in small wool washing plants, upright cylinders are employed, while for continuous large scale working the well known so-called Leviathan apparatus can be utilized. Owing to the intensive solvent action of the cyclohexanones a much improved washing performance is obtained over that of the customary soap process.

Cyclohexanone and its homologues can also be employed with success as solvents in other branches of the textile industry for the purpose of removing fats or oils from textile materials, as, for example, from the spools after spinning yarns, similar advantages exhibiting themselves as in the de-greasing of raw wool.

I claim:

1. Process for the de-greasing of raw wool or other textile material which comprises washing the raw wool or other textile material with a solvent comprising a compound having the general formula:



115  
 120  
 wherein X represents hydrogen or a monovalent aliphatic radicle.

2. Process for the de-greasing of raw wool or other textile material which comprises washing the raw wool or other textile material with a solvent comprising cyclohex-

125  
 130  
 anone.

3. Process for the de-greasing of raw wool or other textile material which comprises washing the raw wool or other textile ma-

terial with a solvent mixture containing a compound having the general formula:

5



wherein X represents hydrogen or a mono-valent aliphatic radicle, and a water-soluble organic solvent having only a relatively small solvent capacity for wool fat and wool wax.

4. Process for the de-greasing of raw wool or other textile material which comprises washing the raw wool or other textile material with a solvent mixture containing a compound having the general formula:

20



wherein X represents hydrogen or a mono-valent aliphatic radicle, a water-soluble organic solvent having only a relatively small solvent capacity for wool fat and wool wax, and a regulated, predetermined small amount of fat.

5. Process for the de-greasing of raw wool or other textile material which comprises washing the raw wool or other textile material with a solvent mixture containing a compound having the general formula:

35



40 wherein X represents hydrogen or a mono-valent aliphatic radicle, and a regulated, predetermined small amount of fat.

6. Process for the de-greasing of raw wool or other textile material which comprises washing the raw wool or other textile

material with a solvent comprising a compound having the general formula:

50



wherein X represents hydrogen or a mono-valent aliphatic radicle, separating at least a part of the solvent from the wool and thereafter washing the wool with an aqueous liquid.

7. Process for the de-greasing of raw wool or other textile material which comprises preliminarily washing the raw wool or other textile material with an aqueous liquid, and thereafter washing the resulting moist wool with a solvent containing a compound of the general formula:

65



wherein X represents hydrogen or a mono-valent aliphatic radicle.

8. Process for the de-greasing of raw wool or other textile material which comprises preliminarily washing the raw wool or other textile material with an aqueous liquid, thereafter washing the resulting moist wool with a solvent containing a compound of the general formula:

70



75 wherein X represents hydrogen or a mono-valent aliphatic radicle, and finally washing the wool with an aqueous liquid.

In testimony whereof, I affix my signature.

80

ALFRED ENGELHARDT.